

Aug. 28, 1962

K. G. COBURN

3,051,587

## METHOD OF TREATING METALLIC STRIP WITH SODIUM VAPOR

Filed Aug. 19, 1960



Fig. 1.

Fig. 3.



Fig. 2.

INVENTOR.  
KENNETH G. COBURN.

Allen · Allen

ATTORNEYS.

## 1

3,051,587

METHOD OF TREATING METALLIC STRIP  
WITH SODIUM VAPORKenneth G. Coburn, Middletown, Ohio, assignor to  
Armco Steel Corporation, Middletown, Ohio, a corpora-  
tion of Ohio

Filed Aug. 19, 1960, Ser. No. 50,722

6 Claims. (Cl. 117—51)

This invention relates to a method of treating metallic strip and the surface of the coating bath with sodium vapor in the coating of ferrous metal strips with aluminum or aluminum alloys by the hot dip procedure.

One of the coating procedures now very generally practiced is one in which the metal strip is first passed through an oxidizing furnace to burn oils and other carbonaceous substances from the surface thereof and to form on the strip a microscopically thin oxide film. The strip is then passed through a reducing furnace in which the thin oxide film is reduced so as to leave the surfaces of the strip absolutely clean, in which state they are particularly receptive to the molten coating metal. The strip is then led through a hood under the protection of a neutral or reducing atmosphere and without a flux treatment into the coating bath. The protective hood dips into the coating bath so that the strip is at no time exposed to the atmosphere. The above outlined procedure is taught in the Sendzimir Patent No. 2,110,893.

When the coating metal is aluminum or an aluminum alloy, difficulties have been encountered in that deposits form on the surface of the aluminum bath and are picked up by the strip and these deposits adversely affect the adhesion of the molten coating metal. This problem was recognized and an antidote therefor was disclosed and claimed in the Oganowski Patent No. 2,437,919. In accordance with the teachings of Oganowski, a bell was provided at the end of the hood which dipped into the coating bath and the bell was provided with an annular trough surrounding the strip and into this trough metallic sodium was fed. Since the trough was subjected to the heat of the bath, the metallic sodium was therefore melted and vaporized.

Oganowski suggested that various substances such as nitrides were formed by the interaction of the bath with the nitrogen of the dissociated ammonia protective atmosphere in the hood and might also include oxides and hydrides formed by the interaction of various substances present with water vapor. He suggested that these nitrides, oxides and hydrides formed a scum on the bath which was dragged down into the bath on the strip which resulted in surface defects.

Oganowski suggested that it was possible to form on the surface of the bath a powdery coating which would be non-adherent to the strip and which would to a very large degree prevent interaction of the bath and atmospheric constituents and in any event render the strip non-adhesive with respect to such nitrides, oxides and the like which might be formed. Oganowski taught that one could form upon a surface of an aluminum bath a layer which consisted mainly of powdery sodium aluminate, by introducing sodium vapors adjacent the surface of the molten aluminum within the hood.

There are certain disadvantages involved in generating the sodium vapor in the hood by the heat of the bath in that the melting and vaporizing temperature is roughly that of the coating bath which is maintained relatively constant. Therefore, sodium vapor is only generated at a constant rate. If it is attempted to add metallic sodium more rapidly, there is a tendency for liquid sodium to splash directly onto the strip and this also produces defects in the coating. Furthermore, when it is remembered

## 2

that the hood contains hydrogen or dissociated ammonia, it will be understood that sodium reacts rapidly with hydrogen to form sodium hydride and therefore the sodium in the trough is rapidly converted to an inactive product so that there is a substantial waste of sodium.

Oganowski suggested that sodium vapors might be generated elsewhere and introduced into the hood, but indicated that this was difficult if not impossible because of the dilution of the sodium vapors by the protective atmosphere and because of the likelihood of turbulence within the hood.

With the foregoing considerations in mind, it is an object of the present invention to provide a method of treating a strip, which is to be coated with aluminum or aluminum alloy, with sodium vapor wherein the sodium vapor is generated outside the hood and is conveyed to the hood by means of a carrier gas. It is another object of the invention to provide for a control of the sodium vapor addition and to provide for greater uniformity in the rate of sodium vapor additions. It is also an object of the invention to eliminate the danger of sodium splash by removing solid and liquid sodium from the immediate vicinity of the strip being coated.

These and other objects of the invention which will be apparent to one skilled in the art are accomplished by that method of which an exemplary embodiment will now be described.

Reference is made to the drawings forming a part hereof and which will illustrate more or less diagrammatically an apparatus by means of which the method may be carried out.

In the drawings,

FIGURE 1 is a diagrammatic view of a vaporizer and coating bath showing the relationship between the two.

FIGURE 2 is a cross-sectional view through an exemplary vaporizer; and

FIGURE 3 is a fragmentary cross-sectional view on the line 3—3 of FIGURE 1.

Briefly, in the practice of the invention there is provided a coating pot which may be conventional with a conventional hood according to the Sendzimir patent, dipping into the molten coating metal and providing a protective passage for the strip from the reducing furnace into the coating bath. A vaporizer is provided with means for heating the vaporizing chamber and means are provided for adding metallic sodium to the vaporizer. A carrier gas is caused to flow into the vaporizer and through the vaporizer, whereby to entrain vaporized sodium and a conduit is provided to carry the carrier gas and its entrained sodium vapor from the vaporizer to the hood.

Referring in greater detail to the drawings, a coating pot is generally indicated at 10 and contains a body of molten coating metal 11. Within the pot there is mounted the usual pot roll 12 around which the strip 13 passes. The hood 14 extends from the exit of the reducing furnace down into the bath 11 and means are provided (not shown) for feeding into the hood a protective atmosphere which will usually be dissociated ammonia. It will be understood that the strip, in passing through the hood 14, has been pretreated so that it is absolutely clean and it then passes into the coating bath, around the pot roll 12 and issues from the bath and is permitted to cool.

In FIGURE 1 a vaporizer is indicated generally at 15. A carrier gas is fed into the vaporizer through a conduit 16 from a suitable source (not shown) and the carrier gas with its entrained sodium vapor passes through a conduit 17 from the vaporizer 15 to the hood 14. Metallic sodium is introduced into the vaporizer through the pipe 18 which is provided with a pair of single action, wide opening valves 19a and 19b. By means of these

valves it is possible to introduce sodium into the vaporizer without sucking air into it.

Referring now to FIGURE 2, the vaporizer comprises a vessel 20 communicating with the pipe 18 and also with the conduits 16 and 17. Electric heating elements indicated schematically at 21 are provided to heat the vessel 20 so that the metallic sodium introduced through the pipe 18 is caused to melt forming a pool of molten sodium 22. Under the influence of the heat provided by the electric heating elements 21, the liquid sodium is vaporized and the balance of the vessel 20 is filled with sodium vapor as indicated at 23. A baffle 24 is provided to cause the carrier gas entering through the conduit 16 to flow downwardly around the baffle, whereby to pick up and entrain vaporized sodium. The carrier gas with the entrained sodium vapor then passes through the conduit 17 which may be heated as by means of heating elements 17, and/or insulated as at 17d, to prevent condensation of the vapor before it reaches the hood.

The vessel 20 is enclosed within an insulating container 25 so as to minimize heat loss and to economize on heat requirements.

As seen in FIGURE 3 where a strip is being coated, the conduit 17 is provided with two branches 17a and 17b preferably entering from opposite sides of the hood and disposed adjacent the surface of the coating bath at a small angle of incidence with respect to the strip so as to cause the sodium vapor to pass across the surface of the bath and the strip with a minimum of turbulence to achieve the results outlined above.

One very important aspect of the present invention resides in the particular carrier gas which is used. It might be thought that because the hood contains dissociated ammonia it would be desirable to use dissociated ammonia as the carrier for the sodium vapor. This, however, is not so because the use of dissociated ammonia results in the formation of sodium hydrides which would tend to plug up the conduit 17.

According to the present invention, the carrier gas used is nitrogen which is completely inert with respect to sodium, and which has the advantage of being heavier than hydrogen so that the hydrogen which is present in the dissociated ammonia atmosphere in the hood is displaced upward by the heavier nitrogen carrier gas. Thus, while a small amount of hydrides may be formed, this hydride formation will be negligible.

It will now be understood that the uniformity of sodium vapor addition may be very accurately controlled by a control of the vaporizing heat applied through the heating elements 21, by the rate of addition of metallic sodium and by the rate of flow of the carrier gas.

Without limitation but by way of example, the above disclosed procedure has been practiced using a temperature between 1000° F. and 1100° F. and a flow of nitrogen of 150 cubic feet per hour. It will be understood that the temperature must be sufficient to heat the carrier gas as well as to provide for the melting and vaporization of the sodium. When the carrier gas is used in large volume, preheating thereof ahead of the sodium vaporizing chamber is advisable, as by means of heating elements 16a.

It will also be clear that by removing the source of the sodium vapor from the hood and the strip passing therethrough, the problem of sodium splash has been entirely eliminated. The use of nitrogen as a carrier gas has eliminated the plugging up of the lines through which

the sodium vapor passes into the hood and build up of frozen metal or high melting point reaction products within the hood has been very greatly reduced. Elimination of the sodium trough of the Oganowski patent permits better heat transfer from the aluminum bath outside the hood, through the metal hood, so as to prevent freezing of the coating metal within the hood. The coating metal sometimes becomes chilled by cold strip or it may have a higher melting point due to iron contamination.

While the use of nitrogen has been described above, it will be understood that other gases which are inert with respect to sodium and sufficiently heavy to displace hydrogen may also be used. Nitrogen is so perfectly adapted for this purpose and is so plentiful and inexpensive that it is the carrier of choice.

It will be understood that various modifications may be made without departing from the spirit of the invention and therefore no limitation not specifically set forth in the claims is intended.

What is claimed is:

1. In a process of coating a ferrous metal article with molten coating metal of a class consisting of aluminum and aluminum alloys, in which the metal article is passed through a hood into a bath of said molten coating metal, and in which a protective atmosphere which is substantially non-oxidizing to ferrous metals is maintained in said hood; the steps of generating sodium vapor outside said hood, conveying said sodium vapor, by means of a carrier stream of nitrogen gas, into said hood adjacent the surface of said molten coating metal, whereby to subject the surface of the molten coating metal and the surfaces of the metal article being coated, to the action of sodium vapor.

2. A process according to claim 1, wherein the protective atmosphere in said hood is dissociated ammonia.

3. A process according to claim 1, wherein the article being coated is a strip of ferrous metal, and said sodium vapor, in its nitrogen gas carrier, is directed at both sides of said strip, adjacent the surface of the molten coating metal, at a small angle of incidence.

4. In a process of coating a ferrous metal article with molten coating metal of a class consisting of aluminum and aluminum alloys, in which the metal article is passed through a hood into a bath of said molten coating metal, and in which a protective atmosphere which is substantially non-oxidizing to ferrous metals is maintained in said hood; the step of continuously subjecting the surfaces of said article and of the molten coating metal within said hood, to the action of sodium vapor entrained in a stream of nitrogen gas.

5. A process according to claim 4, wherein said article being coated is a strip of ferrous metal, and said sodium vapor, in its nitrogen gas carrier, is directed at both sides of said strip adjacent the surface of the molten coating metal, at a small angle of incidence.

6. A process according to claim 4, wherein the protective atmosphere in said hood is dissociated ammonia.

#### References Cited in the file of this patent

#### UNITED STATES PATENTS

|           |            |               |
|-----------|------------|---------------|
| 2,437,919 | Organowski | Mar. 16, 1948 |
| 2,503,571 | Wehe       | Apr. 11, 1950 |
| 2,785,651 | Pawluk     | Mar. 19, 1957 |
| 2,914,419 | Organowski | Nov. 24, 1959 |